

## UNITED STATES PATENT OFFICE

JAMES DRISCOLL, OF PLAINFIELD, NEW JERSEY, ASSIGNOR TO JOHNS-MANVILLE CORPORATION, OF NEW YORK, N. Y., A CORPORATION OF NEW YORK

## FRICITION ELEMENT AND METHOD OF MAKING THE SAME

No Drawing.

Application filed February 21, 1930. Serial No. 430,447.

The present invention relates to an improvement in friction elements having a fibrous asbestos body or base, and in its specific aspect is concerned particularly with an improved friction element having a body portion of woven asbestos yarn.

The invention has as its primary object the provision of a friction element which has a much less tendency to score than the friction elements now available, and the accomplishment of this object without the loss of other desirable qualities such as high tensile strength.

A further object is the provision of a lining of increased density and firmness.

These and other desirable objects are attained according to my invention by incorporating finely divided or powdered zinc with the fibrous asbestos which forms the body or base of the friction element. Although the invention is not restricted to any particular theory of action it is probable that the resulting elimination or very substantial reduction in the tendency of the friction element to score is due to a gradual deposition of zinc from the friction element on to the metallic surface of the drum in the form of an adherent film or coating. The film of zinc thus formed serves to largely prevent the abrasion of metal from the drum and subsequent bedding and coalescence of the same in the friction element, thereby obviating the principal cause of scoring.

While my invention contemplates the improvement of fibrous asbestos friction elements of both the woven and felted types, it is particularly concerned with the provision of an element adapted for use as a brake lining and formed from woven asbestos yarn having powdered zinc incorporated therewith. The zinc powder is preferably incorporated with the yarn by applying a mixture or paste containing the requisite amount of zinc powder to the surface of the yarn prior to the weaving operation. The latter operation may be advantageously effected while the coated yarn is still moist. The coated yarn is then woven into the requisite shape as for instance into a tape or

listing in the usual manner. The woven listing is pressed or calendered and thoroughly dried. The dry listing is then treated according to the usual methods by impregnating with a suitable saturant such as a drying oil, and asphaltic substance or the like, then baked or cured, and calendered to size.

In a specific application of my invention the zinc powder was applied to the yarn in the form of an adhesive mixture or sludge having the following composition by weight:

|                     | Per cent |
|---------------------|----------|
| Bentonite clay----- | 4.28     |
| Water-----          | 47.70    |
| Zinc powder-----    | 47.70    |
| Starch-----         | 0.32     |
|                     | 100.00   |

The bentonite serves as a suspending agent for the zinc but various other known suspending agents may be substituted therefore if desired. The starch serves as an adhesive material and assists in forming an adherent coating of the zinc powder which will not brush off during the subsequent operations. The proportions and ingredients given in this example may be widely varied, the principal requirement being that the mixture contain in suspension, a suitable amount of the zinc powder to form a practically continuous coating on the yarn.

The zinc powder may be incorporated with the yarn in various other ways as for instance by first moistening the yarn with a suitable liquid and then drawing the wet yarn thru a bank of the powdered zinc. The zinc powder may also be incorporated in the finish for asbestos paper and thin strips of the paper thus provided spun into yarn with a wire reinforcement in the usual manner. The zinc powder may also be admixed with the loose asbestos fibers prior to the spinning of the same into yarn. Various other methods of incorporating the zinc powder will occur to those versed in the art. However none of these methods have the specific advantages of the method particularly described herein.

The zinc powder employed is the commercial article sometimes termed zinc dust and is fairly finely sub-divided, for instance, of sufficient fineness to pass thru a 100 mesh to the inch screen.

5 The asbestos yarn is preferably reenforced with a strand of a suitable metal as for example with brass wire. All the yarn entering into the finished fabric may be coated with zinc or only a part thereof depending upon the particular results desired. Excellent results have been obtained by coating only the warps and binders and leaving the fill yarn uncoated.

15 The zinc coating may be advantageously applied to the yarn by causing it to pass thru a bank of the sludge while the yarn is being wound on to beams or bobbins preparatory to the weaving operation.

20 The coated yarn is preferably woven while still moist as any tendency for the coating to brush or peel off is materially reduced thereby. The coated yarn if desired may be braided into the desired shapes, and 25 the term "weaving" as used in the claims includes braiding as well as the conventional weaving operation.

The woven listing is calendered and then completely dried, preferably by heat in an 30 oven. A typical example of the composition of the listing prior to impregnation is as follows:

|                    | Per cent |
|--------------------|----------|
| Brass wire-----    | 19.25    |
| Zinc dust-----     | 18.44    |
| Bentonite-----     | 1.65     |
| Asbestos yarn----- | 60.66    |
|                    | 100.00   |

40 The dried lining may then be impregnated with any suitable saturant. A suitable saturant for instance, is a liquid of the following composition by weight:

|                           | Per cent |
|---------------------------|----------|
| Pitch-----                | 14.00    |
| Blown China wool oil----- | 21.00    |
| Varnoline-----            | 65.00    |
|                           | 100.00   |

50 The saturated lining is then dried and baked or cured in a dry heat oven.

In the production of friction elements having a felted fibrous asbestos base commonly termed mill-board, the requisite 55 amount of zinc powder may be introduced prior to the felting operation by adding it directly to the asbestos pulp.

Friction elements produced according to the above described methods have been 60 found by severe service tests to have a very marked decreased tendency to score brake drums and this advantage is obtained without loss of other desirable qualities. I have found that the introduction of zinc into the 65 friction element in the form of zinc wire re-

enforcement for the yarn is not satisfactory since the strength of the zinc wire is greatly reduced when subjected to the elevated temperatures incident to the processing and use of the friction element. By the 70 combination of zinc powder with asbestos yarn having a wire insertion as for instance brass wire according to my invention, a brake lining is provided having a tensile strength and other desirable qualities equal to the conventional type of brake lining and characterized by a greatly decreased tendency to score brake drums. The improved lining is further characterized by its increased density and comparative firmness 75 which materially reduces the frequency of necessary brake adjustments.

What I claim is:—

1. A method of manufacturing fibrous asbestos friction elements which comprises incorporating powdered zinc with the asbestos in sufficient quantity to substantially reduce the tendency of the element to score during use. 80

2. A method of manufacturing friction elements which comprises incorporating powdered zinc with asbestos yarn and then weaving the yarn into the requisite shape. 85

3. A method of manufacturing friction elements which comprises applying a coating of powdered zinc to asbestos yarn and then weaving the yarn into the requisite shape. 90

4. A method of manufacturing friction elements which comprises coating asbestos yarn with a mixture containing powdered zinc in suspension and then weaving the 95 yarn into the requisite shape. 100

5. A method of manufacturing friction elements which comprises drawing asbestos yarn thru a mixture containing powdered zinc in suspension and then weaving the 105 yarn while still moist into the requisite shape. 110

6. A method of manufacturing friction elements which comprises applying a coating to asbestos yarn of an aqueous suspension of zinc and weaving the yarn into the requisite shape. 115

7. A method of manufacturing friction elements which comprises applying a coating to asbestos yarn of an aqueous mixture containing zinc, a suspending agent therefor and an adhesive material, and then weaving 120 the yarn into the requisite shape. 125

8. A method of manufacturing friction elements which comprises applying to asbestos yarn a coating of a mixture of a colloidal clay, zinc powder and an adhesive material, and weaving the yarn into the requisite shape. 130

9. A method of manufacturing friction elements which comprises applying to asbestos yarn a coating of a mixture of a col-

loidal clay and zinc powder and weaving the yarn into the requisite shape.

10. A friction element comprising a fibrous asbestos base having powdered zinc incorporated therewith in sufficient quantity to substantially reduce the tendency of the element to score during use.

11. A friction element comprising a base of woven asbestos yarn having powdered zinc incorporated therewith.

12. A friction element comprising a base of woven asbestos yarn coated with powdered zinc.

13. A friction element comprising a base of woven reenforced asbestos yarn coated with powdered zinc.

14. A brake lining comprising a base of woven asbestos yarn reenforced with a strand of metal, the surface of said yarn being provided with a coating of powdered zinc.

15. A brake lining comprising a base of woven asbestos yarn reenforced with brass wire, the surface of said yarn being provided with a coating of powdered zinc.

25 Signed at Manville in the county of Somerset and State of New Jersey, this 17th day of February, A. D. 1930.

JAMES DRISCOLL.

loidal clay and zinc powder and weaving the yarn into the requisite shape.

10. A friction element comprising a fibrous asbestos base having powdered zinc incorporated therewith in sufficient quantity to substantially reduce the tendency of the element to score during use.

11. A friction element comprising a base of woven asbestos yarn having powdered zinc incorporated therewith.

12. A friction element comprising a base of woven asbestos yarn coated with powdered zinc.

13. A friction element comprising a base of woven reenforced asbestos yarn coated with powdered zinc.

14. A brake lining comprising a base of woven asbestos yarn reenforced with a strand of metal, the surface of said yarn being provided with a coating of powdered zinc.

15. A brake lining comprising a base of woven asbestos yarn reenforced with brass wire, the surface of said yarn being provided with a coating of powdered zinc.

Signed at Manville in the county of Somerset and State of New Jersey, this 17th day of February, A. D. 1930.

JAMES DRISCOLL.

30

#### CERTIFICATE OF CORRECTION.

Patent No. 1,812,326.

Granted June 30, 1931, to

JAMES DRISCOLL.

It is hereby certified that error appears in the printed specification of the above numbered patent requiring correction as follows: Page 1, line 56, for "and" read an; line 90, for "finish" read furnish; page 2, line 46, for "wool" read wood; and that the said Letters Patent should be read with these corrections therein that the same may conform to the record of the case in the Patent Office.

Signed and sealed this 29th day of September, A. D. 1931.

(Seal)

M. J. Moore,  
Acting Commissioner of Patents.

**CERTIFICATE OF CORRECTION.**

**Patent No. 1,812,326.**

**Granted June 30, 1931, to**

**JAMES DRISCOLL.**

**It is hereby certified that error appears in the printed specification of the above numbered patent requiring correction as follows: Page 1, line 56, for "and" read an; line 90, for "finish" read furnish; page 2, line 46, for "wool" read wood; and that the said Letters Patent should be read with these corrections therein that the same may conform to the record of the case in the Patent Office.**

**Signed and sealed this 29th day of September, A. D. 1931.**

**(Seal)**

**M. J. Moore,  
Acting Commissioner of Patents.**